

May 12, 1931.

E. E. BLAKE

1,804,968

MANUFACTURE OF YARN

Filed Feb. 27, 1929

3 Sheets-Sheet 1



May 12, 1931.

E. E. BLAKE

1,804,968

MANUFACTURE OF YARN

Filed Feb. 27, 1929

3 Sheets-Sheet 2

FIG. 3



FIG. 5



FIG. 4



INVENTOR  
Edmund E. Blake,  
BY  
J. H. McReady,  
his ATTORNEY.

May 12, 1931.

E. E. BLAKE

1,804,968

MANUFACTURE OF YARN

Filed Feb. 27, 1929 3 Sheets-Sheet 3



Fig. 6



Fig. 7

INVENTOR  
Edmund E. Blake,  
BY  
J. H. McCready,  
his ATTORNEY.

## UNITED STATES PATENT OFFICE

EDMUND E. BLAKE, OF SACO, MAINE, ASSIGNOR TO SACO-LOWELL SHOPS, OF NEWTON, MASSACHUSETTS, A CORPORATION OF MASSACHUSETTS

## MANUFACTURE OF YARN

Application filed February 27, 1929. Serial No. 343,127.

This invention relates to methods of and apparatus for working fibrous material into the form of thread or yarn. The invention is more especially concerned with the drawing and spinning of cotton slivers or rovings.

It is the general object of the invention to improve the drawing or drafting of the rovings or slivers in spinning frames with a view both to improving the quality of the resulting thread or yarn and also increasing or lengthening the draft.

In preparing cotton for spinning the fibre first is put through a series of processes designed to free it from dirt and foreign materials, the last of these operations being that of carding. The carding process is also the first of a series of operations designed to bring the fibres into more or less parallel relationship. The cotton comes from the card in the form of a large sliver which must be reduced materially in size before it can be spun. This reduction in size and the straightening and paralleling of the fibres is accomplished in a series of drawing operations, the slivers being doubled between the drafting or drawing processes in order to reduce the irregularities and produce a more uniform and even sliver. Drawing or drafting is, as its name implies, the drawing out of the sliver and it necessarily is accompanied by a reduction in the size of the sliver. It is usually accomplished by running the sliver through successive pairs of rolls, each pair revolving at a greater surface speed than the preceding pair. Before the cotton is ready to go to the spinning frame it is also run through a roving frame and is wound on bobbins. It is necessary to introduce some twist into the slivers in order to give them the requisite strength for winding them on the bobbins and unwinding them again at the spinning frame, and a sliver so twisted is commonly referred to as a "roving." Commonly the twist is from one to five turns per. inch of length according to the fineness of the roving and length of staple. The roving also goes through another very important drawing or drafting operation in the spinning frame immediately prior to being delivered to the spinning instruments, and it is with this drafting operation

that the present invention is especially concerned.

It is obvious that if the length of the draft used in any individual drawing operation could be increased materially, either the number of these operations could be correspondingly reduced or the production of the preparatory machinery be increased; and if the quality of the product could be maintained unimpaired, the cost of preparation of the fibre for spinning would be reduced. Efforts in this direction, however, are hampered by the fact that the fibres in any batch of cotton or in any cotton yarn are not of uniform length. Mixed with the longer fibres are a great number of shorter fibres of various lengths. The fibres are naturally attenuated spirals in form and they have rough surfaces so that when they are drawn over each other in drafting, the shorter fibres are pulled along with the longer ones simply by their contact with them, and this contact is extremely uncertain and variable in character. The ideal condition in drafting would be to have each fibre drawn along in its orderly turn, and while this would be difficult even with fibres of relatively uniform length, it is made vastly more difficult by the presence of the short fibres. In drawing the roving in the spinning frame the drafting operation is further complicated by the presence of the required twist in the roving which tends further to lock the fibres together and therefore to prevent the very action which the drafting mechanism is designed to produce.

A typical drafting mechanism of a type commonly used in spinning frames in this country comprises three pairs of rolls arranged one in advance of the other, with one roll of each pair resting on top of the other, each pair of rolls being driven at a greater peripheral speed than the preceding pair. All three top rolls are usually weighted. The nip of the front pair of rolls is spaced from that of the next pair by a distance very slightly longer than that of the longest fibres, while the distance between the back and middle rolls is usually one and one-quarter inches. The difference in surface speed of the back and middle pairs of rolls is made very small,

the gear or drive ratio usually being between 1.04 and 1.15, and the draft produced between these two pairs of rolls is commonly called the "break draft". Usually it is just enough to straighten out the roving and feed it in a straight line for the main draft which is applied while the roving is being fed from the middle to the front rolls. The main draft, in a typical instance, is in the neighborhood of seven when drawing a single roving.

This arrangement has long been used, and with easy drafts and cotton of fairly uniform staple this three roll mechanism has given reasonably satisfactory results; but any attempt to use a high or long draft with a mechanism of this character on cotton of the usual staple has been found to have a decidedly adverse effect on the quality of the product. Weak places in the roving are drawn excessively and this fact, combined with the difficulty of controlling the shorter fibres, makes for results which are not satisfactory.

It was realized that if the nip of the middle rolls could be brought closer to the nip of the front rolls there would be fewer of these short fibres free from control and that these shorter fibres would be fed to the front rolls in a more regular order. A reduction in this spacing of the front and middle rolls, however, made it necessary to decrease the weight on the top middle roll so as to permit a greater proportion of the length of the long fibres to slip through the middle rolls as they began to be drawn by the faster moving front rolls and thus to avoid breaking them. This, however, resulted in reducing the effectiveness of the middle rolls in producing the break draft. A so-called "four roll" arrangement, therefore, was developed with the idea of producing a break draft between the back and middle rolls, a draft between the two middle pairs of rolls, and then the principal draft between the forward middle and the front pairs of rolls.

A further development dealing with this problem involved the substitution of a belt or apron drafting unit for one or more of the pairs of rolls of the three or four roll drafting mechanisms. In a typical arrangement two belts running in contact with each other, or a belt running in contact with a roll, were substituted for one of the middle pairs of rolls of the three or four roll mechanisms. Typical examples of these belt drafting mechanisms are shown in United States Patents Nos. 1,297,794 and 1,644,747, and in British Patent No. 9,692 of 1915.

The four roll arrangements and some of the belt type drafting mechanisms have proved to be superior to the old three roll constructions, and they perhaps represent the best forms of drafting mechanisms for spinning frames which have been developed prior to the present invention.

In all of the prior arrangements, however,

little or no attention seems to have been given to the proper correlation and arrangement of what I have termed the "break draft elements" in order to produce a satisfactory conditioning of the roving preparatory to the main draft. In fact, in a very large percentage of drafting mechanisms in present use no substantial elongation of the roving or definite preparation of it is produced prior to the application of the main draft. I have found that these factors have a very important bearing on the results produced in the drafting mechanism of a spinning frame, and that superior results can be obtained and substantial economies realized by properly pre-determining and controlling these factors. The present invention, therefore, deals more particularly with the conditioning of the roving, especially the unlocking of the fibres from each other, preparatory to applying the main draft, although it also involves improvements in the main drafting step. It involves improvements both in the methods of and mechanisms for drawing rovings in a spinning frame.

In addition, the invention aims to improve drafting mechanisms of the belt or apron type with a view to producing more uniform results, eliminating difficulties in the guiding, driving and cleaning of the belts, and reducing the care and attention required of mechanisms of this character.

The invention will be readily understood from the following description when read in connection with the accompanying drawings, and the novel features will be more particularly pointed out in the appended claims.

In the drawings,

Figure 1 is a vertical, sectional view from front to rear through the drafting mechanism of a spinning frame constructed in accordance with this invention, much of the mechanism being shown in elevation;

Fig. 2 is a perspective view of a guiding device for the belt tensioning roll;

Fig. 3 is a perspective view of a portion of a spinning frame;

Fig. 4 is a diagrammatic sectional view of the drafting rolls and belt and the mechanism for weighting the rolls;

Fig. 5 is a side elevation of a cap bar;

Fig. 6 is a rear elevation of parts of the mechanism shown in Figs. 1 and 3, and

Fig. 7 is a perspective view of one of the belts and the knurled driving roll for it, a part of the belt being shown broken away.

In this specification the strands of material to be treated will be referred to as "roving" since the fibre ordinarily is in the form of a roving when it is delivered to the spinning frame, and the spun material will be referred to as "yarn".

The drawing mechanism shown comprises a roll stand 2 having suitable bearings in which three driven rolls are mounted, these rolls

being indicated at 4, 6 and 8, respectively. Upper rolls 5, 7 and 9 cooperate with the respective rolls 4, 6 and 8, thus forming three pairs of rolls, namely, front rolls 4—5, middle or intermediate rolls 6—7, and back rolls 8—9. The lower front and rear rolls are of metal and are fluted or grooved in the usual or conventional manner, while the middle lower roll is knurled. The upper rolls are covered with a suitable resilient material, ordinarily consisting of a cloth cot encircling the metal core and an outer leather jacket covering the cot. Each pair of rolls thus is arranged to grip a roving firmly but yieldingly. The resilient covering also has the effect of increasing the area of contact or bite between the individual rolls of each pair and hence improving the effectiveness of the grip of the rolls on the roving while still avoiding any injurious crushing of the fibres. A belt or apron 10 passes between the intermediate rolls 6 and 7 and has a run extending forward toward the front rolls and supported on a stationary bar 12 mounted closely adjacent to the lower front roll 4. From this bar the belt extends downwardly and backwardly around a tensioning roll 14 which is provided with end flanges to limit the lateral movement of the belt relatively to the roll. This roll is mounted to rise or fall and it is guided by two arms 15—15 both pivoted on a rod 16 at the rear of the roll 14, the arms being notched, as indicated at 17—17, to receive the axle or shaft 18 of the roll. Preferably the arms 15—15 are connected rigidly together by a bridge piece 19 which is integral with them so that both arms must move in unison, and the roll 14 thus is kept substantially parallel with the roll 6 which drives the belt. A spring clip 20 sprung over the pivot rod or shaft 16 between the arms 15—15 serves to hold these arms against movement longitudinally of the pivot rod. The belt 10 is tensioned partly by the weight of the roll 14 and partly, also, by the weight of the arms 15—15.

Running on the surface of the belt 10 is a small slip roll 21, relatively light in weight, located between the front and intermediate upper rolls 5 and 7 and directly above the bar 12.

The upper rolls 5 and 9 rest directly on and are driven by their cooperating lower rolls 4 and 8, respectively, but the slip roll 21 and the upper intermediate roll 7 rest on the belt 10 and are driven by their engagement with it, the belt, in turn, being driven by the lower middle roll 6. All of the upper rolls are held in their proper positions by cap bars 22, Figs. 1 and 3, each bar being pivoted at 23, Fig. 1, at the rearward part of the stand so that it can be swung upwardly out of its operative position. The rolls 5, 7, 9 and 21 are provided with reduced ends which rest in slots formed in the sides of the cap

bars 22 and which serve to position the rolls while permitting them to roll freely. It is desirable to be able to adjust the spacing of the intermediate roll 7 toward and from the front roll 5, and for this purpose the cap bar 22 has a rod-like member 24, Fig. 5, extending forward from its main body upon which brackets 25 and 26 are adjustably mounted, the bracket 25 serving to guide the middle roll 7 while the other bracket 26 guides the front roll 5 and the slip roll 21. Screws 27 and 28 serve to hold the respective brackets 25 and 26 in their adjusted positions.

In order to press the upper rolls 5, 7 and 9 firmly against the driven rolls and thus compel the upper and lower drawing elements of each pair to move at substantially the same surface speed, a saddle mechanism is provided which may be of a common type. The construction shown in Figs. 1 and 4 includes a front saddle 30, a rear saddle 31, and a stirrup 32 which is connected to a weighting mechanism of a common type, this mechanism including a lever 33. Pressure so applied to the front saddle 30 is divided between the front roll 5 and the rear saddle 31 and the pressure of the latter is divided about equally between the rolls 7 and 9. The total weight applied may be varied by using different weights on the lever 33.

A long series of drafting units of the character shown in Fig. 1 are supported side by side in a drawing frame and are all operated in unison by driving the lower rolls 4, 6 and 8, the individual roll sections being made on relatively long shafts which are connected together so that they form, in effect, continuous shafts extending the entire length of the frame. Any suitable mechanism may be employed for driving the rolls 4, 6 and 8. A gear mechanism should be used in order to maintain the desired speed relationships between the rolls and to drive the lower rolls positively. The organization of the particular mechanism shown will be obvious from an inspection of Fig. 3 simply with the explanation that the driving gear is shown at 40, the gear 41 is on the end of the roll shaft 6, and the roll shaft 8 is geared directly to the shaft 42. It will be understood that the front rolls are driven faster than the intermediate rolls and the latter revolve faster than the back rolls.

The usual front underclearer or scavenger roll 36 is provided and a top clearer of some kind, such as the roll 35, is used to clean the upper front roll 5.

A unique arrangement has been provided for cleaning the belt 10 and the rear roll 8 and consists of a clearer roll 37 supported to run in contact both with the outer surface of the belt and also with the surface of the roll 8. This clearer is made in relatively long lengths so that one roll cleans the belts and back rolls 8 of a considerable number of

drawing units. It is provided at its ends with gudgeon members, one of which is shown at 38, Fig. 1, and each of these members is supported in a loop 39 formed in a 5 spring 40 which is fastened by a bolt 41 to a part of the stand 2. By depressing the springs 40 which support the opposite ends of any clearer roll 37 or by pushing against it, such roll may be slipped backwardly and 10 upwardly out of the machine. Normally, however, the springs 40 hold the clearer roll against the lower back fluted rolls 8, and it is, therefore, driven chiefly by these rolls, although the belts 10 also tend to rotate the 15 clearer in the same direction that it is revolved by the rolls. Due to the grooved construction of the rolls and the firmer engagement of the clearer with them, they control the movement of the clearer and it revolves 20 at substantially the same surface speed as the rolls. This is slightly slower than the surface speed of the belts and consequently the clearer has a wiping action on the belts which makes it particularly effective.

25 This clearer arrangement represents a substantial improvement over those used heretofore for cleaning the belts of drawing mechanisms in being simpler in construction, more economical to manufacture, more convenient 30 to use, and far more effective. The prior belt drafting mechanisms have used an individual clearer for each belt, and a great deal of trouble has been experienced in keeping these clearers in proper working order. An especially serious difficulty has been the tendency of the fly or lint to collect between the 35 ends of adjacent clearers and to twist into the form of a rope connecting the clearers together these troubles are eliminated in the 40 present construction.

The general organization of the drafting mechanism having been described, certain features of this invention can now be explained which deal especially with the preparation 45 of the fibre for the main drawing operation. Bearing in mind the fact that the roving has considerable twist when it comes to the spinning frame, that the cotton fibres vary in length, have a more or less spiral form 50 with rough surfaces, and are interlocked with each other, it will be clear that if a roving is grasped at two points spaced apart by, say, one and one-quarter inches, (as it would be in an ordinary drawing mechanism), and is 55 pulled at said points, the first effect will be to stretch the roving and to cause the fibres twisted around the outside of the roving to bind all the tighter on the inner fibres. My experiments with the break draft mechanisms 60 of the old three roll constructions have shown that if the roving is not pulled more than, say, 10% of its own length, this will be the only effect produced, and when the pull is released the stretched section of the roving 65 will return or spring back to its original con-

dition. The gear ratio between the two pairs of rolls which produce this break draft in prior art structures is usually between 1.04 and 1.15, and my experiments with such break draft mechanisms show that no net break 70 draft, or, in other words, no permanent elongation of the roving, is produced in normally twisted rovings until a draft of at least 1.10 is applied. Up to this point the roving is simply straightened out to some extent and 75 tensioned.

I have found, however, that if the gear ratio between the pairs of rolls which produce the break draft is increased to in the neighborhood of 1.32 and the rolls are properly spaced 80 from each other and sufficiently weighted, the fibres in the roving are then so unlocked and loosened that an exceptionally long draft can be applied immediately thereafter without adversely affecting the character of the yarn 85 that will be produced. A proper spacing of the rolls, however, is required for this purpose in order to afford the necessary distance or space for the uniform drawing out of the fibres, the partial unlocking of the 90 twist, and the freeing of the individual fibres from each other which occurs after the roving has been fully stretched between the rolls. For ordinary staples and rovings prepared according to the usual American practice I 95 prefer to make this distance in the neighborhood of one and thirteen-sixteenths inches, and the spacing between centers of bites or between roll centers should be at least one and five-eighths inches or, better yet, one and eleven-sixteenths inches and should not ordinarily be more than one and fifteen-sixteenths 100 inches. Too great a space gives unsatisfactory results due apparently to the loss of control of the fibres and the tendency to draw 105 weak points excessively.

While, as above stated, a gear ratio of approximately 1.32 on ordinary commercial rovings and with usual staples produces the best results, this gear ratio can be made anywhere from 1.27 to 1.37 without seriously affecting the results, and can even be reduced to 1.20 or raised to 1.45, and still, with the proper spacing of the rolls, produce results 110 decidedly superior to those obtained in the prior art structures. The proper spacing of the break draft rolls is an important factor in obtaining these improved results. Tests have shown that the net break draft obtained, or, in other words, the permanent elongation 115 of a normally twisted roving, with these gear ratios and spacings is not equal to the full difference in surface speed of the so-called "gear draft", but that there is a loss due to the elasticity and straightening of the roving. The gear ratio preferably is made such that 120 the permanent elongation of the roving produced in this part of the mechanism is in the neighborhood of from 18% to 25%. With such a net break draft produced with drafting 125 130

elements spaced as above described, the fibres are unlocked from each other, and the grip introduced by the twist is effectually released so that the roving then is exceptionally well prepared for the application of the main draft. So far as I am aware, the importance of so conditioning a roving for the main draft has not been appreciated heretofore, nor have the elements of drafting mechanisms been so arranged and correlated as to produce such preparation effectively.

The main or principal draft is applied by the action of the front rolls 4 and 5 in taking the fibres as fed to them. As the roving passes between the intermediate rolls it comes in contact with the belt 10, and it is carried forward with the belt under the slip roll 21. This roll cooperates with the belt to maintain the fibres, especially the shorter fibres, under control as they move toward the nip of the front rolls and while they are being drawn by the front rolls. Since the roll 21 rests on the belt and is rotated thereby at substantially the speed of the belt, it does not tend to draw the fibres, but it assists in keeping the shorter fibres under better control while allowing the longer fibres to slip under it and over the belt as these fibres are drawn forward by the front rolls. It acts, also, to restrain the tendency of the shorter fibres to move with the longer fibres simply due to their haphazard contact, and to cause the feeding or drawing of these shorter fibres in their regular turn. This is essential to the production of an even uniform yarn made from cotton of usual staple.

The action which takes place between the front and middle rolls is quite different from that which occurs between the middle and rear rolls. As above stated, a relatively small draft is produced between the rear and middle rolls and the drawing action which does take place at that point is, generally speaking, a mass drawing of the entire roving for a very short distance, while that which occurs between the front and middle rolls is intended to draw out the individual fibres in their orderly turn. In the preparatory or conditioning draft the first action is to straighten out and to stretch the roving as a whole, this action tending to contract the roving and to some extent to bind the fibres together due to the presence of the twist. I have found that when a normal roving is gripped firmly between the rear rolls, a zone of influence of the twist extends forward for the greater part of the distance toward the intermediate rolls, and that the drawing action which is produced here is confined chiefly to a relatively short zone lying immediately back of the intermediate rolls, although a movement of the longer fibres takes place for a very considerable distance back of these rolls due to their length. The chief purpose of the draft applied here is to unlock the

fibres and partially free them from each other and from the twist, although it is desirable to leave a certain amount of twist in the roving because it assists in controlling the fibres subsequently during the main draft. In the latter draft the front rolls grip the fibres firmly, and because their surface speed is very much higher than that of the middle roll, they draw the fibres out and reduce the roving to the desired size and condition for spinning.

Control of the fibres during the main draft is influenced materially by the remaining twist and by the spacing of the intermediate rolls with relation to the front and slip roll. Preferably the slip roll 21 is run as close to the upper front roll as practicable, and the center of the slip roll is spaced from the center of the middle roll by approximately fifteen-sixteenths of an inch, or slightly less, seven-eighths of an inch usually being the preferred distance for staples of less than one and one-quarter inches. If the slip roll is made half an inch in diameter the distance between the centers of the rolls 5 and 7 will be approximately one and five-eighths inches. These distances and dimensions have been found to produce good results, although it will be understood that they may be varied somewhat. In fact, in running staples of approximately one and one-quarter inches or more it is desirable to set the middle top roll back slightly and this can readily be done, even while the machinery is running, by adjusting the blocks 25, as above described.

While the roll spacing above mentioned seems relatively short, it is permitted by the fact that the roving has been properly conditioned for the main draft and it is of advantage in the better control which it affords of the short fibres. In other words, it leaves a minimum of space in which the short fibres can be drawn along solely by fibre contact.

I have found that in order to enable the slip roll 21 to perform its functions properly its weight is an important factor. Preferably it should weigh in the neighborhood of 1200 grains and this weight should not be departed from by over 200 grains plus or minus if the best results are to be secured.

I have found, also, that it is advisable to apply more pressure on the upper, back and middle rolls than has been the usual practice in order to obtain more certain and reliable results. In the mechanism shown rolls of the ordinary size can be and preferably are used. Each of the upper rolls is of approximately fifteen-sixteenths of an inch in outside diameter and has two "bosses" or working surfaces to act on the fibre, the bosses usually being about one and three-eighths inches in length. In a spinning frame of two and three-quarters inch gage and bosses of the size just mentioned, I have obtained excellent results by applying a pressure of

from 32 to 34 pounds to the stirrup 32 and so adjusting the distribution of this weight that approximately 14 to 16 pounds is applied on the front roll 5 and the remainder is equally divided between the intermediate and rear rolls 7 and 9. As above stated, each roll has two working surfaces or bosses and these surfaces are separated by a reduced portion or "neck" on which the saddle members act so that the pressure applied to each roll is equally divided between the two working surfaces or bosses of the roll. It is preferable for ordinary staples and twists not to reduce these pressures applied to the back and middle rolls more than two pounds. Such pressures with rolls constructed as above described give a positive grip on either a single or double roving but will not injure the fibre because of the resilient character of this grip.

The drafted roving passes directly from the bite of the front rolls to the spinning instrumentalities which twist it to produce yarn, the fibre being fed continuously through the drawing mechanism and to the spinning apparatus.

The method and apparatus herein described have been found in actual practice to produce very substantial advantages over prior art structures and processes. A stronger, evener and more uniform yarn can be made while still using a draft which would be too high for ordinary drawing mechanisms. Or, the draft can be increased very substantially while still producing a yarn of as good a quality from a given staple as is produced by the standard mechanisms. Several factors contribute to these improved results, such as the better conditioning of the roving for the main draft, the fact that the majority of the fibres are kept under better control, and the fact that the small portion of fibres of maximum length are not injured or broken as usually occurs in feeding the ordinary staple through the usual drafting mechanisms. This conserves the very considerable strengthening action which these few longer fibres, if preserved, add to any yarn.

The length of the main draft necessarily will depend upon the length and body of the staple, the characteristics of the roving, and the results desired. I have found that entirely satisfactory results can be produced by using a main draft equal to 2, plus 1 for each sixteenth of an inch of length of staple. In other words, for a seven-eighths inch staple a draft of 16 is entirely satisfactory, while for a one and one-quarter inch staple a main draft of 22 gives superior results. Under favorable conditions and with longer staples the draft can be run up considerably higher, for example, from 25 to 30, but perhaps with some sacrifice of quality. If quality is the fundamental consideration a draft

of in the neighborhood of 16 is more likely to be used on ordinary staples. With these higher drafts the roving fed to the drawing mechanism of the spinning frame can be relatively large or coarse for a given size, "count", or "number" of yarn. This means that an economy in the preparation of the yarn for spinning can be realized. Or the mechanism can be used to produce a higher quality of yarn from a given fibre.

A further advantage of this drawing mechanism is that it is unnecessary to make any changes in the setting of the bottom rolls for very substantial variations in staple. I have successfully run the range of staples from seven-eighths up to one and five-eighths inches in length without such changes. It is also unnecessary to make any change in the apparatus for the ordinary variations in twist in the roving.

While I have herein shown and described a typical embodiment of my invention, it will be understood that the invention may be embodied in other forms and that the method of the invention may be practiced with other mechanisms without departing from the spirit or scope thereof.

Having thus described my invention, what I desire to claim as new is:

1. The herein described method comprising the steps of subjecting a cotton roving to a preliminary draft by grasping it firmly between moving drafting elements at points spaced at least  $1\frac{1}{16}$  inches apart, driving said elements at a ratio of between 1.20 and 1.45 and thereby feeding the roving through them while they draw it, next subjecting said roving to a main draft, then spinning the roving so drafted and passing the roving continuously from the first of said drafting operations to the next and from the latter to the spinning operation.

2. The herein described method comprising the steps of subjecting a cotton roving to a preliminary draft between successive pairs of drafting elements driven at a ratio of between 1.20 and 1.45 and which firmly grip the roving at points spaced at least  $1\frac{1}{16}$  inches apart, then subjecting said roving to a much greater draft by passing the same between drafting elements which move at a surface speed substantially the same as that of the preceding pair of elements and which grip the roving with a light pressure while it is drawn out by additional drafting elements that move at a relatively high speed, and then passing the drafted roving to spinning instrumentalities.

3. The herein described method comprising the steps of subjecting a cotton roving to a preliminary draft between drafting elements adapted to firmly grip the roll at points spaced from  $1\frac{1}{16}$  inches to  $1\frac{1}{8}$  inches apart and having a driving ratio of between 1.20 and 1.45, next subjecting said rov-

ing to a main draft while maintaining the shorter fibres under control, then spinning the roving so drafted, and passing the roving continuously from one of said drafting 5 operations to the next and from the latter to the spinning instrumentalities.

4. The herein described method comprising the steps of providing a cotton roving which is relatively coarse for the size of 10 thread to be made from it, subjecting said roving to a preliminary draft which permanently elongates the roving from 18% to 30%, then subjecting said roving to a main draft sufficient to reduce the roving to the 15 size desired for the yarn to be spun, holding the greater part of the fibres under control during said main draft, then spinning the roving so drafted, and passing the roving continuously from one of said drafting 20 operations to the next and from the latter to the spinning instrumentalities.

5. That improvement in methods of making cotton yarn which consists in subjecting a cotton roving to a preparatory treatment 25 by passing the same between successive pairs of drawing rolls which firmly grip the roving at points spaced at least  $1\frac{1}{16}$  inches apart, driving said rolls at such surface speeds as to produce a permanent elongation 30 of said roving of at least 18%, then subjecting the roving so prepared to a main draft sufficient to reduce it to the desired size for spinning, finally spinning the roving so drawn to form a yarn, and passing said roving continuously from one of said drafting steps to the next and from the latter to the spinning 35 operation.

6. That improvement in methods of making cotton yarns which consists in subjecting 40 a cotton roving to a preparatory treatment by passing the same between successive pairs of drawing rolls, the bites of which are spaced apart from one and eleven-sixteenths inches to one and seven-eighths inches, driving said 45 rolls at such surface speeds as to produce a permanent elongation of said roving of between 18% and 27% of its own length, then subjecting the roving so prepared to a main draft sufficient to reduce it to a suitable size 50 for spinning, finally spinning the roving so drawn to form a yarn, and passing said roving continuously from one of said drafting steps to the next, and from the latter to the spinning operation.

55 7. That improvement in methods of preparing cotton fibre for spinning which consists in subjecting a cotton roving to a preparatory treatment by passing the same between successive pairs of drawing rolls constructed to firmly but 60 yieldingly grip the roving and having their bites spaced on centers from  $1\frac{1}{16}$  inches to  $1\frac{1}{8}$  inches apart, driving said rolls at such surface speeds as to produce a permanent elongation of said roving of between 18% and 30%, and immedi- 65

ately thereafter subjecting the roving so prepared to a draft of at least 1 for each sixteenth of an inch of length of the staple.

8. That improvement in methods of making cotton yarn which consists in subjecting 70 a cotton roving to a preparatory treatment by passing the same between successive pairs of drawing rolls constructed to firmly but yieldingly grip the roving and having their bites spaced from  $1\frac{1}{16}$  inches to  $1\frac{1}{8}$  inches apart, driving said rolls at such surface speeds as to produce a permanent elongation of said roving of between 18% and 30%, then subjecting the roving so prepared to a draft 75 of at least 10, next spinning the roving so drafted, and passing the roving continuously from one of said drafting steps to the next and from the latter to the spinning operation.

9. A drawing mechanism for spinning frames comprising, in combination, front, 80 back and intermediate pairs of drafting elements, each adapted to grip a roving firmly between them, means for supporting said elements in their operative positions, the centers of the bites of said intermediate and back 85 elements being spaced at least  $1\frac{1}{16}$  inches from each other, and mechanism for driving said lower elements to produce a drive ratio between said rear and intermediate elements of from 1.20 to 1.45 and a substantially 90 higher drive ratio between said intermediate and front elements.

10. A drawing mechanism for spinning frames comprising, in combination, front, 100 back and intermediate pairs of drafting rolls, each pair comprising an upper and a lower roll for gripping a roving firmly between them, means for supporting said rolls in their operative positions, the centers of the bites of said intermediate and back rolls being spaced 105 at least  $1\frac{1}{16}$  inches from each other, a belt passing between said intermediate rolls and having a run extending forward toward the bite of said front rolls, means located closely adjacent to the lower of said front rolls for supporting said belt at the forward end of its run, a slip roll resting on said belt between said front and intermediate rolls, and mechanism for driving all of said lower 110 rolls to produce a drive ratio between said back and intermediate rolls of between 1.20 and 1.45, and a substantially higher drive 115 ratio between said intermediate and front rolls.

11. A drawing mechanism for spinning frames comprising, in combination, front, 120 back and intermediate pairs of drafting rolls, each pair comprising a lower roll and a resilient upper roll, means for supporting said rolls in their operative positions and holding said intermediate and back rolls with their bites spaced on centers between  $1\frac{1}{16}$  inches and  $1\frac{1}{8}$  inches apart, a belt passing between said intermediate rolls and having a run extending toward the bite of said front 125 130

rolls, a stationary bar located closely adjacent to the lower of said front rolls and supporting said belt at the forward end of its run, a slip roll resting upon said belt above said bar closely adjacent the top front roll, mechanism for driving all of said lower rolls to produce a drive ratio between said back and intermediate rolls of from 1.20 to 1.45 and a substantially higher drive ratio between said intermediate and front rolls, and means for applying a pressure of at least six pounds on each of said upper, front, intermediate and back rolls.

12. A drawing mechanism for spinning frames comprising, in combination, front, back and intermediate pairs of drafting rolls, each pair comprising an upper and a lower roll, means for supporting said rolls in their operative positions and holding said intermediate and back rolls with their bites spaced on centers between  $1\frac{5}{8}$ ths inches and  $1\frac{15}{16}$ ths inches from each other, a belt passing between said intermediate rolls and having a run extending toward the bite of said front rolls, a stationary bar located closely adjacent to the lower of said front rolls and supporting said belt at the forward end of its run, a slip roll weighing between 1,000 and 1,400 grains and resting on said belt between said front and intermediate rolls, mechanism for driving all of said lower rolls positively to produce a drive ratio between said rear and intermediate rolls of from 1.20 to 1.45 and a substantially higher draft between said intermediate and front rolls, and means for pressing the upper of each of said pairs of rolls toward its respective underlying roll to firmly but resiliently grip a roving fed between said three pairs of rolls.

13. A drawing mechanism for spinning frames comprising two pairs of drawing rolls arranged one in advance of the other, each pair comprising an upper and a lower roll, mechanism for driving said front rolls at a greater surface speed than the rear rolls, a belt passing between said rear rolls and having a run extending forward toward the bite of said front rolls, said belt also including a loop lying below said rolls, a tensioning roll in the lower part of said loop having flanges at its opposite ends to limit the lateral movement of said belt with reference to the roll, and means for guiding said tensioning roll.

14. A drawing mechanism for spinning frames comprising, in combination, front, back and intermediate pairs of drafting rolls, each pair comprising an upper and a lower roll for gripping a roving firmly between them, means for supporting said rolls in their operative positions, the centers of the bites of said intermediate and back rolls being spaced at least  $1\frac{5}{8}$ ths inches from each other, a belt passing between said intermediate rolls and having a run extending forward toward the

bite of said front roll, means located closely adjacent to the lower of said front rolls for supporting the belt at the forward end of its run, a slip roll resting on said belt between said upper, front and intermediate rolls, said slip roll being located closely adjacent to said upper front roll and bearing on said belt at a point spaced between thirteen-sixteenths and fifteen-sixteenths of an inch from the point at which said upper intermediate roll bears on said belt, and mechanism for driving all of said lower rolls to produce a driving ratio between said back and intermediate rolls of between 1.20 and 1.45 and a substantially higher drive ratio between said intermediate and front rolls.

15. A drawing mechanism for spinning frames comprising two pairs of drawing rolls arranged one in advance of the other, each pair comprising an upper and a lower roll, mechanism for driving said front rolls at a greater surface speed than the rear rolls, a belt passing between said rear rolls and having a run extending forward toward the bite of said front rolls, said belt also including a loop lying below said rolls, a gravity belt tensioning roll in the lower part of said loop having flanges at its opposite ends to limit the lateral movement of the belt with reference to the roll, and pivoted arms located at the opposite ends of said tensioning roll for guiding and weighting the roll.

16. A drawing mechanism for spinning frames comprising in combination, front, back and intermediate pairs of drafting rolls, each pair comprising an upper and a lower roll, a belt passing between said intermediate rolls and having a run extending forward toward the bite of the front rolls and a loop extending downwardly below said rolls, a removable clearer roll running in contact both with the outer surface of said belt and also with the surface of said lower back roll, and means for supporting said clearer roll in its operative position.

17. A drawing mechanism for spinning frames comprising, in combination, front, back and intermediate pairs of drafting rolls, each pair comprising an upper and a lower roll, a belt passing between said intermediate rolls and having a run extending forward toward the bite of the front rolls and a loop extending downwardly below said rolls, a tensioning roll in said loop, arms pivoted at the rear of said belt and engaging the shaft of said tensioning roll at opposite sides of the belt, said arms serving to guide and weight the roll, a clearer roll running in contact both with the outer surface of said belt and also with the lower of said back rolls, and yielding means for holding said clearer roll in its operative position.

18. In a drawing mechanism, the combination of a series of drafting units arranged side by side, each unit comprising a plurality

of pairs of drafting elements spaced apart and arranged to act successively on a roving to draw it, one of said pairs of elements including a belt, means for driving said units in unison, a single clearer roll for cleaning the belts of a plurality of said units, and means for removably supporting said roll in its operative position.

19. In a drawing mechanism, the combination of a series of drafting units arranged side by side, each unit comprising a plurality of pairs of drafting elements spaced apart and arranged to act successively on a roving to draw it, one of said pairs of elements including a belt, means for driving said units in unison, a single clearer roll for cleaning the belts of a plurality of said units, and means for revolving said roll independently of said belts.

20. 20. In a drawing mechanism, the combination of a series of drafting units arranged side by side, each unit comprising a plurality of pairs of drafting elements spaced apart and arranged to act successively on a roving to draw it, one of said pairs of elements including a belt, means for driving said units in unison, a single clearer roll for cleaning the belts of a plurality of said units, and means for driving said roll at a different

30 surface speed from that of said belts.

21. In a drawing mechanism, the combination of a series of drafting units arranged side by side, each unit comprising a belt and a plurality of pairs of drawing rolls, means for driving said units in unison, and a clearer roll engaging the belts of a plurality of said units and also engaging one of the rolls of the latter units and arranged to be driven by such engagement.

40 EDMUND E. BLAKE.

45

50

55

60

65